

## UNITED STATES PATENT OFFICE

2,121,204

## BEARING METAL ALLOY

Edward P. Langworthy, Rochester, N. Y., assignor to Bearium Metals Corporation, Rochester, N. Y., a corporation of New York

No Drawing. Application November 18, 1936,  
Serial No. 111,491

1 Claim. (Cl. 75—159)

This invention relates to an antifriction metal, proposing an alloy suitable for substantially universal application as a bearing metal and having components which will readily unite in such proportions as may be most suitable for each particular use.

Heretofore, tin has been considered as one of the essential components of alloys of the character generally described. When employed in relatively small quantities, i. e. less than 10%, this metal will, if other factors (which are variable and difficult of control) are favorable, unite with the other components to form a solid solution. However, if a percentage of tin greater than the order of 10% be employed, the tin will be thrown out of solution as the mixture cools and will unite with one of the components to form a substance which in many respects is similar to a eutectoid alloy. For example, when copper is one of the components the excess tin combines with it, the substance thus produced being so much harder than the matrix metal that it is unsuitable for the purpose in view. The maximum percentage of tin which can be employed without the formation of such a substance is variable, depending, among other factors, upon the elements which form the alloy, the temperature at which the molten metal is poured and the rate at which it is permitted to cool. The percentage of tin necessary to impart the desired properties to the alloy may be, however, and in many instances is, substantially greater than that which will remain in solution. In such cases, of course, a lower percentage of tin than is desirable must be employed. On the other hand, the percentage of tin required may be within a range in which it is impossible, without performing tests, to determine whether all of it will remain in solution. Tin, therefore, is satisfactory only when the proportion which is necessary to impart the desired properties to the alloy is less than that at, or above, which the tin will be thrown out of solution.

The principal object of the invention is to overcome the above objections, this object contemplating an alloy of the character generally described which does not involve the use of tin and wherein each component will readily form a union with the remaining components throughout the entire range of proportions which may be necessary to modify the characteristic properties of the alloy in accordance with the particular environment under which it is to be employed.

A further object is to provide a bearing metal whose components, as to proportions, are prede-

termined in accordance with the physical characteristics of the parts which contact with, and which are movable relatively to, the said metal.

A still further object is to provide a bearing metal which will prevent excessive wearing or scoring of the shaft or other associated part in the event that there is a failure in the supply of the lubricating medium to the cooperating surfaces.

The invention contemplates a bearing metal consisting of copper, lead and nickel in the following proportions: copper from 45% to 77%; lead from 20% to 35%; and nickel from 3% to 15%.

The specific percentage selected in each of the ranges noted is determined by the environment in which the metal is to be used, it being preferred that the bearing metal in each case be slightly softer than the metal of the shaft or other part which is to be associated with it in order that if the friction between the parts becomes excessive, owing to a failure in the supply of the lubricating medium to the cooperating surfaces, or for any other reason, the bearing metal will take up the increased wear, thereby preventing injury to the said shaft or other part. The alloy is rendered softer by increasing the percentage of lead or by decreasing the percentage of nickel, or both, and is rendered harder by decreasing the percentage of lead or increasing the percentage of nickel, or both. Assuming, for example, that the alloy which is to be produced is to be formed into bearings for shafts of relatively soft steel, the percentage of lead which is selected will be near the upper limit of the range indicated. The percentage of nickel, although relatively low, will be as high as is permissible, the greater part of the desired degree of softness preferably being attained, when this is possible, by the use of a high percentage of lead rather than by a low percentage of nickel in order that the adhesive characteristic of the copper will be counteracted while the antifrictional properties of the alloy will be substantially increased. A relatively high percentage of nickel has the advantage that the compression and tensile strength of the alloy are correspondingly high. On the other hand, if the alloy which is to be produced is to be formed into bearings for shafts of relatively hard steel the percentages of the alloy components are selected so that the metal of the bearings will be relatively hard, although slightly softer than that of said shafts, it being preferred that, if possible, the greater part of the increase in hardness of the alloy be attained in such case

45

50

55

60

65

70

75

80

85

90

95

by increasing the nickel content rather than be decreasing the lead content in order to retain in as large a degree as possible the high anti-frictional properties inherent in the lead.

5 It will be apparent from the foregoing that the invention contemplates a bearing metal having components which may be used in such proportions as will insure an alloy which will be relatively softer than the shaft or other part with 10 which it is to be employed. It is preferred, however, that in each case the bearing metal be only slightly softer than such shaft or other part, the proportions of the alloy components being selected so that the softness, or hardness, of the 15 bearing metal is correlated to that of the said shaft or other part. As each component of the bearing metal described will readily unite with the others in amounts which will enable the attainment of this end, maximum compression and 20 tensile strength and high antifrictional properties are insured for each environment of use.

The bearing metal has the further advantage 25 that scoring or marring of the shaft or other associated part will be prevented even though there may be a failure in the supply of the medium which is utilized to lubricate the cooperating surfaces. If for this reason, or for any other reason, the friction between the cooperating surfaces becomes excessive the only surfaces scored or

marred, if any are scored or marred, will be those provided by the bearing metal.

The alloy may be produced in any suitable manner. The preferred practice is to heat in a crucible, or otherwise, ingots having a copper 5 content of 50% and a nickel content of 50% together with copper which is added in an amount which will bring the total copper content of the mixture up to the desired percentage. After the ingots and added copper have melted they form 10 a solution, the copper being the solvent and the nickel the solute. The lead, preferably molten and substantially pure, is then introduced into the crucible, it being understood that the lead may, if desired, be introduced in a solid state. 15 The lead is not in solution but is in suspension, the particles thereof being uniformly dispersed throughout the molten solution and being assisted incidentally by the nickel in maintaining their positions in the solution. 20

I claim as my invention:

An alloy for providing a bearing which is capable of preventing excessive wearing or scoring of the shaft or other associated part in the absence of a lubricating medium, said alloy containing 25 45% to 77% copper, 20% to 35% lead and 3% to 15% nickel, the sum of the percentages of copper, lead and nickel equaling substantially 100%.

EDWARD P. LANGWORTHY.